# EUROPEAN PATENT SPECIFICATION

(11) **EP 0 276 081 B1**
(45) Date of publication and mention of the grant of the patent: **30.10.1991**
(21) Application number: 88300258.6
(22) Date of filing: 13.01.1988
(51) Int. Cl.: C10G 1/00

(54) **Process for preparing a normally liquid hydrocarbon product from plastics material**
Verfahren zur Herstellung eines unter Normalbedingungen flüssigen Kohlenwasserstoffproduktes aus Kunststoffmaterial
Procédé de préparation d'un produit hydrocarburé normalement liquide à partir d'un matériau plastique

(30) Priority: 20.01.1987 JP 9160/87
(43) Date of publication of application: 27.07.1988
(73) Proprietor: MOBIL OIL CORPORATION, New York New York 10017 (US); DIRCTOR GENERAL OF THE AGENCY OF INDUSTRIAL SCIENCE AND TECHNOLOGY, Chiyoda-ku Tokyo (JP); RESEARCH DEVELOPMENT CORPORATION OF JAPAN, Kawaguchii, Saitama 332 (JP); K.K. FUJI TECH, Shiso-Gun Hyogo Prefecture (JP)
(72) Inventor: Saito, Kiyoshi The Government Ind. Dev. Laboratory, Toyohira-ku Sapporo City Hokkaido (JP); Fukuda, Takashi The Government Ind. Dev.Laboratory, Toyohira-ku Sapporo City Hokkaido (JP); Suzuki, Satoru The Government Ind. Dev. Laboratory, Toyohira-ku Sapporo City Hokkaido (JP); Sato, Hideo, Fukayasu-gun Hiroshima Prefecture (JP); Hirota, Toshio, Yokohama City (JP)
(74) Representative: Colmer, Stephen Gary

(56) References cited:
- EP-A- 0 101 291
- US-A- 4 423 265
- US-A- 4 584 421

## Description

The present invention relates to a process for preparing from a plastics material a normally liquid hydrocarbon product which is useful, into alia, as a raw material for the production of gasoline.

As the quantity of plastics manufactured has grown in recent years, disposal of plastics scrap has become an increasing problem. Moreover, although various thermal cracking methods have been proposed as potential solutions to the disposal problem, they are disadvantageous in that formation of a considerable amount of coke and waxy materials, which tend to adhere to the inner wall of the reaction vessel, is unavoidable. Accordingly, it has not been feasible to put these methods to practical use in the disposal of commonly used plastics.

One alternative proposal for treating plastics scrap is disclosed in the U.S. Patent No. 4584421 and involves initially subjecting the scrap to thermal decomposition and then contacting the resultant vaporous product with a catalyst, such as a natural zeolite, at a temperature of 350-470°C. However, this process suffers from the problems that the zeolite catalyst undergoes rapid aging and the product is of high molecular weight so as to be useful only as a heavy fuel.

The present invention resides in a process for preparing a normally liquid hydrocarbon product, that is comprising C₅-C₂₂ hydrocarbons, which comprises thermally cracking a plastics material in the molten liquid phase and catalytically converting the vaporous product thereby generated by contact at 200-350°C with a zeolite having a constraint index between 1 and 12.

The plastics material used in the process of the invention may be any polymer or copolymer of an ethylenically unsaturated monomer, including aromatic species such as polystyrene and polyethylene terephthalate, although halogen-containing polymers and copolymers should be avoided. Preferably, the material is a polyolefinic plastics material, especially polyethylene, polypropylene and polybutylene (including copolymers and mixtures containing the same as an essential component). Since the present process is specifically intended for the disposal of scrap plastics, the plastics material employed may take a wide variety of forms, such as, films, sheets, and moldings, although films and sheets are preferred. These materials, after being pulverized by appropriate means, are fed continuously to a thermal cracking reactor by means of an extruder while being heated to a liquid and molten state.

The thermal cracking step of the process of the inventon is conducted with the plastics material in the molten liquid phase. The temperature employed in the thermal cracking step is preferably 390-500°C, more preferably 400-450°C, and the pressure is preferably atmospheric. It is preferred continuously to feed the plastics material to the thermal cracking step so that the level of the molten liquid phase in the cracking reactor is maintained substantially constant. The thermal cracking reaction is preferably carried out with stirring and in the presence of an inorganic porous particulate material. Whereas there is no particular limitation for the nature and size of the inorganic porous particulate material, provided that it is not deformed or deteriorated, it is usually preferably to employ porous particulate material having a size of about 1-10 mm. Illustrative embodiments of suitable porous particulate materials are natural zeolites, bauxite and red mud (residue remaining after removal of aluminum from bauxite). The porous particulate material may exhibit some cracking activity although this should be lower than that of the zeolite catalyst used in the subsequent catalytic conversion step.

Use of the inorganic particulate, material assists heat transfer during thermal cracking, inhibits attachment of coke to the reaction vessel, and lowers the boiling point of the vaporous product formed, thereby facilitating supply of the vaporous product to the catalytic conversion step and improving the quality and yield of the finally produced hydrocarbon oil. The amount of the inorganic particulate material is preferably at least 5% by weight, but can be up to 200-400% by weight, of the molten material in the reaction tank.

The paraffin-rich vaporous product formed in the thermal cracking step is then passed to a catalytic conversion unit containing a zeolite having a constraint index between 1 and 12. The term constraint index is defined in, for example, U. S. Patent No. 4,016,218. Examples of suitable zeolites include ZSM-5 (see U.S. 3702886), ZSM-11 (see U.S. 3709979), ZSM-12 (see U.S. 3832449), ZSM-23 (see U.S. 4076842), ZSM-35 (see U.S. 4016245) and ZSM-48 (see U.S. 4375573), although ZSM-5 is preferred. The zeolite is normally employed in its hydrogen form, although it may contain a metal such as platinum. The zeolite is also usually combined with a binder, such as alumina, and formed into particles having a size of 0.1-10 mm.

The catalytic conversion reaction is normally carried out at atmospheric pressure, WHSV of 0,8-0.85 and a temperature of 200-350°C, preferably of 250-340°C. The operation at such low temperature is unexpected and not only achieves economic advantages but also inhibits undesirable side reactions.

Use of the zeolite in the second cracking step not only allows a decrease in the cracking temperature and continuous operation but also improves the quality and yield of the product. Aging of the zeolite catalyst is found to be relatively slow and the present process can be conducted with a zeolite catalyst which has been regenerated after use in this or another reaction.

The resultant product is a hydrocarbon oil of low pour point demonstrating the occurrence not only of the cracking reaction but also of isomerization reactions. Absence of high molecular weight substances in the product is also evident. In fact, the hydrocarbon oil product contains only in substantial amounts of hydrocarbons having more than 22 carbon atoms. The hydrocarbon oil product can therefore be added directly to the gasoline blending pool. Gaseous by products are also obtained in the present process but these contain a substantial proportion of valuable C₃-C₅ compounds.

The invention will now be described below with reference to the accompanying drawing, which is a diagrammatic illustration of apparatus for performing a method according to one example of the invention.

Referring to the drawing the thermal cracking reactor is indicated generally at 1 and includes a feed supply zone 2, a thermal cracking reaction zone 3 and a stirrer 4 mounted on top of zone 3. The feed supply zone 2 supplies a screw feeder 5 which in turn feeds plastics material into the top of the thermal cracking reaction zone 3. Inside the thermal cracking reaction zone 3 are inserted a level meter 6 to measure height of the molten feed and a thermometer 7.

The top of the thermal cracking reactor 1 is connected to a catalytic reaction zone 8 which is filled with HZSM-5 having a particle size of about 3 mm into which is also inserted a thermometer 9. The bottom of the thermal cracking reactor 1 is provided with a gas burner 10.

The thermal cracking reaction zone 3 is maintained at the desired operating temperature by the burner 10, whereas the catalytic reaction zone 8 is maintained at its operating temperature by means of the heat capacity of the vaporous thermal cracking product, although an external heater (not shown) may also be employed.

The effluent from the catalytic reaction zone 8 is fed by way a cooling tube 12 equipped with a water-cooling condensor 11 to oil storage tanks 13 and 14 for collection.

In one practical embodiment, the apparatus shown in Figure 1 was constructed and operated as follows:
(A) The screw feeder 5 was of the two-axis screw type and was operated at a temperature of 330°C and a supply rate of 680-706 g/hr.
(B)The thermal cracking reactor 1 was a cylindical tank 560 mm in height, 105 mm in diameter and 4.85 liter in volume. The thermal cracking reaction zone 3, namely, the molten liquid phase area of the reactor 1, was 250 mm in height, was filled with 250 g of natural zeolite produced in Kasaoka, Japan (particle size of approximately 0.5 mm) and was stirred at 8 rpm.
(C) The catalytic cracking reaction zone 8 was a cylindincal tower 300 mm in height, 76 mm in inner diameter and 1.36 liter in volume and was filled with 613 g of ZSM-5 in the hydrogen form.

The invention will now be more particularly described in the following Examples.

### EXAMPLE 1

Polyethylene film, obtained as urban waste, was collected and pulverized to a size of approximately 5 mm. The pulverized feed was placed in the feed supply zone 2, heated to melting in the screw feeder 5 and fed to the first stage, thermal cracking reaction zone. The vaporous product thereby generated was passed to the second stage catalytic reaction zone 8 in which catalytic conversion was carried out. The conditions employed and the results obtained are summarized in the following table:

Analysis of a typical hydrocarbon oil product gave the following results:

- Saturates: 38.4%
- Olefins: 54.7%
- Aromatics: 4.5%
- RON(clear): 62.5%

Analysis of a typical gaseous by-product of the process of gave the following results as a percentage basis of the entire gaseous component:
H₂ 7.0: CH₄ 8.0; C₂H₄ 4.5; C₂H₆ 7.6;
C₃H₈ 5.6; C₃H₆ 19.9; i-C₄H₁₀ 1.1;
n-C₃H₁₀ 9.8; i-C₄H₈ 24.5; i-C₅H₁₂ 0.5;
n-C₅H₁₂ 11.5.

Typical material balances were as follows:

### EXAMPLE 2

The process of the preceding Example was repeated with two separate feeds, one consisting of particulate polyethylene and the other consisting of a particulate mixture of 90 wt% polyethylene and 10 wt% polystyrene. The results obtained are summarized as follows:

## Claims

1. A process for preparing a normally liquid hydrocarbon product which comprises thermally cracking a plastics material in the molten liquid phase and catalytically convertion the vaporous product thereby generated by contact at 200-350°C with a zeolite having a constraint index between 1 and 12.

2. The process according to Claim 1 wherein the vapor phase catalytic conversion is effected at a temperture between 250 and 340°C.

3. The process according to Claim 1 or Claim 2 wherein the molten liquid phase thermal cracking is effected in the presence of an inorganic porous particulate material.

4. The process according to Claim 3 wherein the inorganic porous particulate material has catalytic cracking activity.

5. The process according to Claim 4 wherein the inorganic porous material is a naturally occurring zeolite.

6. The process according to any proceeding Claim wherein the liquid phase thermal cracking is effected at a temperature in the range between 390 and 500°C.

7. The process according to any preceding Claim 1 wherein the zeolite used in the catalytic conversion step is ZSM-5.

8. The process according to any preceding claim wherein the plastics material is a polyolefinic plastic material.

9. The process according to Claim 8 wherein the polyolefinic plastics material is a homo- or copolymer of ethylene, propylene or butene.

10. The process according to any preceding Claim wherein the liquid product of the vapor phase catalytic conversion is substantially composed of hydrocarbons having carbon numbers not more than 22.

## Patentansprüche

1. Verfahren zur Herstellung eines unter Normalbedingungen flüssigen Kohlenwasserstoffproduktes, das das thermische Cracken eines Kunststoffmaterials in der geschmolzenen, flüssigen Phase und die katalytische Umwandlung des dadurch erzeugten, dampfförmigen Produktes durch Kontakt mit einem Zeolith bei 200 bis 350°C umfaßt, der einen Zwangsindex von 1 bis 12 aufweist.

2. Verfahren nach Anspruch 1, worin die katalytische Umwandlung der Dampfphase bei einer Temperatur von 250 340°C durchgeführt wird.

3. Verfahren nach Anspruch 1 oder 2, worin das thermische Cracken der geschmolzenen, flüssigen Phase in Gegenwart eines anorganischen, porösen, partikelförmigen Materials durchgeführt wird.

4. Verfahren nach Anspruch 3, worin das anorganische, poröse, partikelförmige Material eine katalytische Crackativität aufweist.

5. Verfahren nach Anspruch 4, worin das anorganische, poröse Material natürlich vorkommender Zoelith ist.

6. Verfahren nach einem der vorstehenden Ansprüche, worin das thermische Cracken der flüssigen Phase bei einer Temperatur im Bereich von 390 bis 500°C durchgeführt wird.

7. Verfahren nach einem der vorstehenden Ansprüche, worin der beim katalytischen Umwandlungsschritt verwendete Zeolith ZSM-5 ist.

8. Verfahren nach einem der vorstehenden Ansprüche, worin das Kunststoffmaterial ein polyolefinisches Kunststoffmaterial ist.

9. Verfahren nach Anspruch 8, worin das polyolefinische Kunststoffmaterial ein Homo- oder Copolymer von Ethylen, Propylen oder Buten ist.

10. Verfahren nach einem der vorstehenden Ansprüche, worin das flüssige Produkt der katalytischen Umwandlung der Dampfphase im wesentlichen aus Kohlenwasserstoffen zusammengesetzt ist, die Kohlenstoffzahlen von nicht mehr als 22 aufweisen.

## Revendications

1. Un procédé de préparation d'un produit hydrocarboné liquide dans les conditions normales qui comprend le craquage thermique d'un matériau plastique en phase liquide fondue et la conversion catalytique du produit sous forme vapeur ainsi obtenu par contact à 200 à 350°C avec une zéolite ayant un indice de contrainte compris entre 1 et 12.

2. Le procédé selon la revendication 1, dans lequel la conversion catalytique en phase vapeur est effectuée à une température comprise entre 250 et 340°C.

3. Le procédé selon la revendication 1 ou 2, dans lequel le craquage thermique en phase liquide fondue est effectué en présence d'un matériau particulaire poreux inorganique.

4. Le procédé selon la revendication 3, dans lequel le matériau particulaire poreux inorganique a une activité de craquage catalytique.

5. Le procédé selon la revendication 4, dans lequel le matériau poreux inorganique est une zéolite d'origine naturelle.

6. Le procédé selon l'une quelconque des revendications précédentes, dans lequel le craquage thermique en phase liquide est effectué à une température de 390 à 500°C.

7. Le procédé selon l'une quelconque des revendications précédentes, dans lequel la zéolite utilisée dans l'étape de conversion catalytique est la ZSM-5.

8. Le procédé selon l'une quelconque des revendications précédentes, dans lequel le matériau plastique est un matériau plastique polyoléfinique.

9. Le procédé selon la revendication 8, dans lequel le matériau plastique polyoléfinique est un homo- ou un copolymère d'éthylène, de propylène ou de butène.

10. Le procédé selon l'une quelconque des revendications précédentes, dans lequel le produit liquide de l'étape de conversion catalytique en phase vapeur est sensiblement composé d'hydrocarbures ayant un nombre de carbones qui n'est pas supérieur à 22.
